

No. 762,914.

PATENTED JUNE 21, 1904.

R. KRON, JR.

MANUFACTURE OF ROLLS OF SHORT FIBER MATERIAL SUITABLE FOR  
TWISTING AND SPINNING.

APPLICATION FILED DEC. 6, 1902.

NO MODEL.



Fig. 1.



Fig. 3.



Fig. 2.

Witnesses:

Henry Thorne

George Barry Jr.

Inventor:

Rudolf Kron, Jr.

by attorneys

Brown, Reward

## UNITED STATES PATENT OFFICE.

RUDOLF KRON, JR., OF GOLZERN, GERMANY.

## MANUFACTURE OF ROLLS OF SHORT-FIBER MATERIAL SUITABLE FOR TWISTING AND SPINNING.

SPECIFICATION forming part of Letters Patent No. 762,914, dated June 21, 1904.

Application filed December 6, 1902. Serial No. 134,201. (No specimens.)

*To all whom it may concern:*

Be it known that I, RUDOLF KRON, Jr., a citizen of the Republic of Switzerland, and a resident of Golzern, Kingdom of Saxony, German Empire, have invented new and useful Improvements in the Manufacture of Rolls of Short-Fiber Material Suitable for Twisting and Spinning, of which the following is a specification.

10 This invention relates to the manufacture from short-fiber asbestos, cellulose, and similar materials of rolls, which I term "magazine-rolls," from which the material may be drawn off in strips suitable for spinning, twisting, and the like; and it consists both in the novel process hereinafter described of producing such a roll and in the roll so produced.

According to this process the asbestos or 20 other short-fiber material is macerated or reduced to a pulp or paste, and this is "formed" into a broad endless web in a similar manner to that adopted in paper-making. Firmness is imparted to this web by draining, suction, 25 pressing, and drying. The resulting web of material while in its pulpy condition is furrowed in the direction of its length at suitable intervals in its width and to such depth as to nearly divide it into a large number of 30 narrow strips and is then drained and pressed or otherwise deprived of water and dried sufficiently, but so that it still contains a suitable degree of moisture to enable the strips which are produced by separating the web in 35 the furrows to be spun moist. For the purpose of thus furrowing the web a number of fine sprays or jets of liquid, steam, or air may be caused to impinge upon the web of pulp as this is formed and carried forward on a 40 woven-wire, felt, or other forming-surface, the distance apart of these sprays or jets corresponding to the desired breadth of the strips.

In order to prevent the partly-formed strips of pulp or material from floating apart under 45 the action of the jets or sprays and to insure the preservation of their proper relative positions, a powerful suction apparatus is disposed below the web. The jets or sprays which produce the dividing-furrows are projected under a very high pressure and are of

great fineness, so that the furrows produced are so fine that in the subsequent pressing and partial drying of the web they become practically closed, while the fibers of the material which connect the intervening strips 55 are nevertheless so readily separable that a slight pull suffices to draw off the strips from the apparently uniform and undivided web.

In the accompanying drawings, Figure 1 represents a perspective view of a magazine-roll, which and the process for obtaining it 60 constitute my invention; and Fig. 2, a plan, partly in section. Fig. 3 shows, on a larger scale, in section, the web with the furrows for forming the undivided strips. 65

The web *a* coming from the screen of a paper-making machine is wound on a core or mandrel *b*.

*c* represents the furrows provided in the manner described above either during or after the formation of the web *a*. The strips from the breadth of the web can be divided or separated by a cutting action, as shown at *d*, so that shorter magazine-rolls are obtained, which are contained together on the core or 70 mandrel *b*. In the example shown a shorter magazine-roll consists of five small strips subdivided by furrows. From such a shorter magazine-roll, which may be slipped from the core or mandrel *b*, the separate strips can be 75 drawn off by a very little pull to supply them to the spinning, twisting, spooling machines 80 and the like.

I claim—

1. The process herein described for manufacturing magazine-rolls of short-fiber material from which strips may be supplied to a spinning, spooling or twisting machine in a moist condition, said process consisting in forming from a pulp of the short-fiber material an adherent broad endless web, furrowing said web in the direction of its length at suitable intervals in its width and rolling the so-furrowed web in the form of a solidly-compact roll from which the strips may be drawn 95 off one or more at a time.

2. The process herein described for manufacturing magazine-rolls of short-fiber material from which strips may be supplied to a spinning, spooling or twisting machine in a 100

- moist condition, said process consisting in forming from moist pulp of the short-fiber material an adherent broad endless web, furrowing said web in the direction of its length at suitable intervals in its width, partially drying said web and rolling the so-furrowed and partially-dried web in the form of a solidly-compact roll from which strips may be drawn off one or more at a time.
10. 3. As a new improved article of manufacture magazine-rolls of short-fiber material in moist condition, consisting in a rolled, adherent broad endless web formed from moist pulp of the short-fiber material furrowed dur-

ing its formation on the screen of a paper-machine in the direction of its length at suitable intervals in its width and partially-dried, from which magazine-roll strips may be drawn off one or more at a time.

In testimony that I claim the foregoing as my invention I have signed my name, in presence of two witnesses, this 17th day of November, 1902.

RUDOLF KRON, JUNIOR.

Witnesses:

JOSÉ M. CERAUDE,  
R. URGOETI.